

# UNITED STATES PATENT OFFICE.

CARL AUER VON WELSBACH, OF VIENNA, AUSTRIA-HUNGARY, ASSIGNOR TO WELSBACH LIGHT COMPANY, OF GLOUCESTER CITY, NEW JERSEY, A CORPORATION OF NEW JERSEY.

## MANUFACTURE OF ELECTRIC FILAMENTS.

976,527.

Specification of Letters Patent. Patented Nov. 22, 1910.

No Drawing.

Application filed August 9, 1898. Serial No. 688,202.

*To all whom it may concern:*

Be it known that I, Dr. CARL AUER VON WELSBACH, a subject of the Emperor of Austria-Hungary, residing at Vienna, Austria-Hungary, have invented or discovered a certain new and useful Improvement in the Manufacture of Electric Filaments, of which the following is a specification.

My invention relates to the production of a dense, coherent metallic filament for incandescent electric lamps, consisting of metallic particles fritted together, and which incandesces at a temperature above that at which platinum volatilizes.

It had been known that osmium possessed several of the prerequisites for this purpose but owing to its utter lack of ductility it has heretofore been impossible to form it into incandescent filaments. It is exceedingly brittle, and therefore its particles cannot be depended upon for mutual adhesion (as can the particles of other metals; platinum, for instance,) to permit of the forming of a wire by ordinary processes. Moreover, while it has been recognized that osmium is a good conductor of electricity, yet it was not known that it was non-volatile *in vacuo* or certain protective gases at temperatures far above the temperatures at which platinum volatilizes.

I have discovered that, at very high temperatures, in an atmosphere of certain protective gases, or *in vacuo*, it is possible to obtain a commercial osmium filament composed of the metal in a partially fused or cinder-like condition and wherein the particles are in intimate contact sufficient to obtain perfect electric conductivity and the requisite flexibility and elasticity for the uses intended, while at the same time the filament resists liquefaction even at such high temperatures. This maintaining of its solid form, when the heating is effected in the presence of certain gases or in a vacuum such as that of the ordinary electric lamp, and the refusal to liquefy or volatilize, continue up to temperatures much higher than that at which the volatilization of platinum occurs; a fact which is utilized as one of the bases of the present invention.

To fully understand my invention, it must be remembered that the metal osmium (among those of its group of highly infu-

sible metals) is peculiar in that it oxidizes with great readiness, when in the presence of free oxygen.

According to my present method, I employ an inner carrier or fillet upon which osmium is deposited, after which I remove the inner carrier or fillet by the heat of an electric current, in the presence of suitable gases, and cause the particles of osmium to assume a partially fused or cinder-like condition, producing an elastic wire of coherent particles of osmium. The thickness or cross section of the filament is determined by the capacity of the osmium filament to support itself after the removal of the carrier or fillet upon which it has been formed, and also by the degree of electrical resistance which is required. That is to say, it should be as thin as possible, to have proper resistance, and thick enough to sustain itself, and capable of withstanding shocks and jars to which it is subjected when in use. The cross section of the filament is also dependent upon other conditions present, such as its length and the purity of the osmium employed.

I will now describe a method which may be followed in making filaments of the kind to which this invention relates, although it will be understood that I do not restrict myself to the precise steps or materials, inasmuch as equivalents for both can be readily substituted by those acquainted with this art.

I first procure an organic thread or threads (I prefer vegetable threads) of fine fibers, which should not be too strongly twisted together, inasmuch as the pores or interstices should be as open as possible for the reception of the coating or impregnating mass.

I make a mixture of any of the sulfids of osmium (which although more or less insoluble in water can be suspended therein in an exceedingly fine state of subdivision) with a small quantity of suitable binding material, such as sugar. The whole is brought to a cream-like consistency by the addition of a suitable quantity of water. The ingredients are thoroughly incorporated so that the osmium sulfid may be uniformly distributed throughout the mass. I then immerse the thread or threads or coat them with this composition until they are thor-

oughly permeated or coated thereby. When fine threads are employed (because of the possibility of thorough impregnation) two or more thereof can be to advantage twisted, 5 woven or interlaced together so as to form a composite thread or fabric which shall be of sufficient cross section to result in a filament of the required dimensions. This weaving, lacing or twisting should occur 10 after the threads have been impregnated or coated with the composition, and to render the thread or threads more uniform they may be drawn while moist, through a die or subjected to the action of a suitable mold, 15 to give a uniform cross section and consequently a uniform resistance throughout. After being sufficiently impregnated or coated and shaped as desired, the threads are dried, and are then subjected to dry dis- 20 tillation. The threads thus prepared are thereafter placed in an electric circuit and heated to a point at which the carbon is eliminated and the reduction of the osmium compound occurs. To assist in such reduc- 25 tion and preserve the metallic osmium, use is made of a suitable reducing atmosphere, as for instance the gases from a "flashed back" Bunsen burner, which contain hydro- 30 gen, carbon-dioxid, carbon monoxid, hydro- carbons and water vapor. The function of the water vapor is to remove the carbon by oxidation and to form with it an inert gas. After the removal of the carbon I then carry 35 the heat to a point at or beyond that at which platinum volatilizes to complete the cementation or cohesion of the particles of metallic osmium.

Having completed the foregoing treatment, it will be found that the metallic 40 osmium has assumed a thread-like form and is coherent throughout and of sufficient flexibility and elasticity to adapt it for use as an incandescent electric filament. The filaments thus produced are readily distinguish- 45 able in that they are devoid of carbon, have the necessary flexibility and resiliency or elasticity, and depend upon metallic osmium not only for their conductivity, but for the incandescence which is produced at a tem- 50 perature at which platinum would be volatilized.

I have mentioned sulfid of osmium as one of the compounds which I can employ, but I wish it to be understood that substitutions 55 can be made therefor of any suitable compounds of this metal, as, for instance, the tetroxide or the metal itself in a finely divided condition, can be used.

Now while I have set forth one method 60 and certain materials which can be employed, I wish it to be understood that I do not limit myself to that precise method or to the materials specified, as my invention includes the use of both ruthenium and 65 rhodium in the place of osmium, and

methods which are substantially the equivalent of that herein set forth.

While ruthenium and rhodium can be substituted for osmium and treated in the same manner for the production of an incandescent filament, yet such filaments are by no means as effective as those of osmium, since both ruthenium and rhodium although melting at temperatures higher than platinum melt at temperatures much below that of osmium. Alloys of osmium, ruthenium, and rhodium may also be used. The efficiency of the filament however, depends upon its withstanding extremely high temperatures and temperatures above that at which platinum volatilizes.

To the composition to be used, may be added certain of the refractory rare earths, such as thoria, zirconia, and the ytterite earths. If, at the termination of the treatment of the filament in the reducing atmosphere, it is found that it is not of uniform resistance throughout its entire length, the requisite equal conductibility may be obtained by surrounding it again with an atmosphere of the same reducing gases and vapor, and again highly heating the filament by the electric currents and from time to time introducing small quantities of volatile osmium compounds, as for instance, osmium tetroxid. The filaments are now ready for mounting in the ordinary incandescent bulbs which should be thoroughly exhausted or filled with inert gases when ready for use.

In the course of my experiments, I have devised other methods for the manufacture of my osmium filament which are set forth in an application for Letters Patent filed herewith, Serial No. 688,201, and wherein I have made claim specifically to my within described, dense, coherent, compact osmium filament which incandesces at a temperature at which platinum would volatilize.

What I claim herein is:

1. The herein described method of manufacturing incandescent electric filaments, consisting in associating organic thread with osmium; then, subjecting the thread to dry distillation; and then, by the action of the electric current, in a suitable atmosphere eliminating the carbon and uniting the metallic particles into a coherent filament of metallic osmium; substantially as set forth.

2. The herein described method of manufacturing incandescent electric filaments, consisting in associating organic thread with osmium chemically combined with another substance to form a reducible compound and thereafter subjecting the same to dry distillation; then, by the action of the electric current in a suitable atmosphere eliminating the carbon and reducing the said compound to the metallic state; and then, causing the uniting of the metal particles

into a dense, coherent, compact and flexible filament of metallic osmium; substantially as set forth.

3. The herein described method of manufacturing an incandescent electric filament of metallic osmium, consisting in associating organic thread with osmium and subjecting the thread to dry distillation; and then placing the same in a suitable atmosphere wherein, by the action of the electric current the carbon is eliminated, whereby the metallic particles of osmium are united into a coherent filament of metallic osmium, substantially as set forth.

10 4. The herein described method of manufacturing a metallic electric filament, consisting in associating organic thread with metal having a higher point of fusion than that of platinum, and, subjecting the same

to dry distillation, and placing the same in a suitable atmosphere wherein the carbon is eliminated, and by the action of the electric current at a temperature at which platinum would volatilize, causing the metallic particles to unite into a dense, compact, 25 coherent filament suitable for electric incandescence; substantially as set forth.

5. A dense, coherent metallic filament for incandescent electric lamps, consisting of metallic particles fritted together and which incandesces at a temperature above that at which platinum volatilizes; substantially as set forth.

Signed this 27th day of July 1898.

CARL AUER VON WELSBACH.

Witnesses:

LUDWIG HAITINGE,  
ADOLF GALLIA.